

# United States Patent Office

2,854,338

Patented Sept. 30, 1958

1

2,854,338

## NEGATIVE WORKING DIAZO SULFONATE FOILS

Clifford E. Herrick, Jr., Chenango Forks, and Ann H. Balk, Woodstock, N. Y., assignors to General Aniline & Film Corporation, New York, N. Y., a corporation of Delaware

No Drawing. Application March 18, 1955  
Serial No. 495,358

9 Claims. (Cl. 96—75)

The present invention pertains to a negative working diazo sulfonate foil in which the diazo sulfonate is imbibed to a layer of a mixture of a maleic anhydride-vinyl compound copolymer and a hydrophobic resin compatible therewith, said copolymer having been treated to produce water sensitivity for application of the diazo sulfonate and the utilization of such a foil in the preparation of colored copies of good actinic opacity.

It has been recognized that diazotype materials containing diazo sulfonate, unlike other diazotype materials, have the peculiarity when exposed under a pattern and developed by means of an alkali of yielding an image opposite in character to that in the pattern. Thus, if the image in the pattern is negative, that produced in the diazotype material will be positive, and vice versa. Although this fact has been known for years, no satisfactory negative working diazo sulfonate process has ever been commercially developed. In this connection, reference is made to the article by Van der Grinten entitled, "The Diazotype Printing Process," which appears in the Photographic Journal, vol. 92B, 1952, pages 43 et seq., in which Van der Grinten, in paragraph 3 of page 43 states:

"Neither the negative diazotype process of the type of Dr. West's process, the earliest diazotype process of all, nor that of the type of the Feer process which is based on the use of diazosulphonates, have been commercialized despite the interest the latter had raised for copying from continuous tone negatives, followed by re-copying on positive diazotype materials and for use in making multicolour pictures."

It is believed to be self-evident that the possibilities inherent in the diazo sulfonate procedure have much to recommend it. The very fact that the art has failed to realize these potentialities underlines the problems which the commercial use thereof entails. These, it may be said, center mainly around the inability of prior operators to produce a carrier for the diazo sulfonate which would meet commercial standards.

The negative working diazotype materials were initially made by utilizing, as the carrier for the sensitizer, a surface-saponified layer of cellulose acetate. More recently, there was employed as such carrier a hardened gelatin coated foil or paper. The utilization of these water sensitive materials, however, presents serious obstacles. Thus, the surface-saponification of cellulose acetate is a difficult technical procedure for the reason that it involves the repeated application of a saponifying solution together with adequate neutralizing and washing operation to remove excess caustic. The saponifying solution generally consists of an alkaline water-organic solvent mixture which must be carefully controlled with respect to the concentration of all components during use. This necessarily means that saponification is not only difficult but expensive.

Similarly, the application of gelatin to a transparent base, such as cellulose acetate, is an involved procedure requiring complicated subbing techniques, elaborate coat-

ing and driving facilities and, in general, all the equipment and technical knowledge required in preparing photographic filmbase. Furthermore, washed gelatin layers require long periods of drying before they can be handled without danger of marring the surface. For this reason they present no advantages over photographic materials. Finally, gelatin, when hardened by use of formaldehyde or chromic salts, loses much of its water sensitivity upon aging, making it difficult to effect a complete washout of unused chemicals.

It has now been found that a commercially satisfactory negative working diazo sulfonate foil can be prepared by coating on a transparent base, a layer of a maleic anhydride-vinyl compound copolymer mixed with a compatible hydrophobic resin, treating the maleic anhydride copolymer to effect splitting, which may include partial amidification of the maleic anhydride linkages, and sensitizing the resulting water sensitive layer with a coating solution containing a diazo sulfonate and a coupling component. The material produced in this way contains a low-cost, easily processed, water sensitive layer which is dimensionally stable, permits ready washout of chemicals, is easily handled when wet, and dries very quickly after processing. Such materials have unexpectedly superior properties from the standpoint of printing speed, opacity to actinic rays and especially improved stability. In fact, it is possible for the first time by use of such foils to place the negative working diazo sulfonate process on a commercial scale, while permitting the selection of a printing system with such foils to insure the obtainment of prints having an improved continuous or dot tone or a controlled contrast and gradation and lacking the grain found in photography.

Negative working diazo sulfonate foils containing a carrier layer rendered water sensitive as above and the processing of such foils by exposure under a pattern and development with a base to produce a negative or positive copy having, if desired, an improved continuous or dot tone or a very high contrast or controlled gradation constitute the purposes and objects of the present invention.

Our diazo sulfonate foil is realized by first dissolving a mixture of a maleic anhydride-vinyl compound copolymer and a compatible hydrophobic resin in an organic solvent to yield a solution suitable for coating. The proportions of copolymer to resin by weight may vary from at least 1:6 to 6:1 with excellent results. The lacquer solution is coated on a transparent base and dried down to form an essentially hydrophobic layer.

If reduction in curl is a desideratum the back side of the base is coated with an organic solvent, such as acetone, methyl Cellosolve, methyl Cellosolve acetate, formic acid and the like, and again dried.

The film is next subjected briefly to the action of a water soluble base to effect hydrolysis of the maleic anhydride linkages of the copolymer. Due to such hydrolysis, water sensitivity is imparted to the layer thus making it capable of taking up the sensitizing components from aqueous solution.

The sensitizing components comprising the light sensitive diazo sulfonate, coupling component and other usual adjuncts are now applied to the water sensitive layer from an aqueous solution. After drying, the material is ready for use and may be exposed to actinic light under a negative photographic transparency and developed in ammonia vapors to produce a positive image. Conversely, by exposing under a positive, a negative image is obtained. Residual diazo sulfonate is removed from the unexposed areas and the backgrounds cleared by a brief washing in hot or cold water. Providing the sensitizing components have been selected for actinic opacity, any

washing in hot or cold water. Providing the sensitizing components have been selected for actinic opacity, any

number of diazotype reproductions may be made from this intermediate foil with no significant darkening of the foil background.

Copolymers of maleic anhydride with vinyl compounds and their preparation are well known in the art and, in this connection, reference may be made to Reissue Patent 23,514, granted June 24, 1952. Any of the copolymers of this patent may be employed in the preparation of our foils. Preferably, however, we use a copolymer of maleic anhydride with a vinyl ether, such as methyl vinyl ether, 2-methoxyethyl vinyl ether, 2-ethoxyethyl vinyl ether, isobutyl vinyl ether and the like. Similarly, while the proportions of the components of the copolymers may vary as indicated in the patent, we have found that best results ensue when utilizing equimolecular quantities of the monomeric components.

Any hydrophobic resin compatible with the copolymer may be employed and, in this connection, reference is made to the cellulose esters and mixed esters, such as cellulose acetate, cellulose propionate, cellulose acetate propionate, nitrocellulose and polyvinyl resins, such as polyvinyl acetate, polymethyl-methacrylate and the like.

The solvent employed for making the lacquer solution of copolymer and resin may be any organic solvent capable of effecting dissolution of the components involved. Such solvents include acetone, butyl acetate, dioxane, tetrahydrofuran, ethyl methyl ketone, cyclohexanone and mixtures thereof with methyl Cellsolve and the like.

The quantity of solvent to copolymer and hydrophobic resin will vary depending upon the solvent used and the components to be dissolved therein. It may be stated, however, that the proportions must be such as to yield a solution of a viscosity suitable for coating. Manifestly, such viscosity may be determined by a simple test.

The hydrolysis of the copolymer is effected by the use of a water soluble base either in the vapor or liquid state. For instance, hydrolysis may be effected by a brief exposure of the film to ammonia fumes or, on the other hand, hydrolysis may be achieved by immersion in an alkaline solution of a water soluble base, such as ammonium hydroxide, or an alkylolamine, such as 2-aminoethanol, 2-dimethylaminoethanol and the like. Hydrolysis is allowed to proceed to such an extent that the layer becomes water sensitive and capable of taking up the sensitizing solution.

The sensitizing solution, essentially comprising the light sensitive diazo sulfonate and a coupling component, may be applied by immersion or by any other technique used in the diazotype art. Any light sensitive diazo sulfonate previously suggested for the negative working method may be employed, but we prefer to use such light sensitive diazo sulfonates as p-ethoxybenzenediazosulfonate; p-methoxybenzenediazosulfonate; 2,5-dimethoxybenzenediazosulfonate and the like.

The particular coupling components employed are not critical and those usually recommended for light sensitive diazotype materials have been found satisfactory. Examples of such couplers are resorcinol; phloroglucinol; tetrahydroxybiphenyl; dichlororesorcinol; dihydroxybiphenyl and 1-(5-hydroxy-1-naphthyl)biguanide. Examples of other couplers that may be employed will be found in the Van der Grinten article referred to above.

The transparent base to which the copolymer hydrophobic resin is applied may be any of the usual transparent bases employed in the diazotype field. The only limitation on the base is that it be transparent and that it provide good wet and dry bonding between itself and the layer coated thereon. Preferably, we utilize a plastic material, such as cellulose acetate or higher acetylated celluloses.

It has been stated that the essential components of the sensitizing solution are the diazo sulfonates and the coupling components, but it is to be understood that the sensitizing solutions may contain the usual adjuncts em-

ployed in the manufacture of light sensitive diazotype materials. These include metal salts for intensification of the dyestuff image, such as ammonium sulfate, nickel sulfate, zinc chloride and the like; stabilizing agents such as thiourea, thiosinamine, sodium salt of o-sulfonybenzaldehyde, naphthalenetrisulfonic acid and the like; acids acting to retard premature dye formation such as citric acid, boric acid, tartaric acid and the like; hygroscopic agents, such as glycol, glycerin and the like, and wetting agents, such as saponin, lauryl sodium sulfonate or the like.

The negative sulfonate process produces images of soft toe characteristics, and as a consequence it is possible to obtain some improvement in the appearance and gradation of the diazotype images produced by such process. However, it is often desirable when working with our diazo sulfonate foil to realize prints which have a good continuous tone or, conversely, prints having a very high contrast. We have ascertained, and this is an important feature of our invention, that improvement in the continuous tone properties may be obtained to a marked extent if the original negative silver image is copied onto our diazo sulfonate foil and the foil is then copied onto a positive working diazotype material such as a diazo foil or print material. Prints made in this sequence, to wit, silver negative  $\rightarrow$  diazotype intermediate negative diazo sulfonate foil  $\rightarrow$  diazotype diapositive or print produce distinctly better gradation in both the toe and highlight regions of the print. In this particular use, our diazo sulfonate foil is capable of yielding copies which have good continuous tone behavior in both highlight and shadow regions.

In the event that prints of very high contrast are desired, the above printing system may be modified so that the original silver negative is printed onto a positive working diazotype foil, the latter onto our intermediate diazo sulfonate foil, and said intermediate onto a positive working light sensitive material, such as a light sensitive diazotype positive or a light sensitive photographic positive. The final printing step, to wit, that involving the diazo sulfonate foil and the light sensitive positive material affords the great advantage of printing with the sensitized surfaces of the involved materials in contact. When proceeding in this fashion, we have found that the line contrast is excellent, although continuous tone is, of course, sacrificed.

The soft sensitometric toe typical of the prints obtained with negative diazo sulfonate foils has previously been commented upon. This characteristic may create difficulties in certain applications. It is possible, however, to increase the low density contrast of our negative foils by placing a bleach-out layer in front of the diazo sulfonate image-forming layer, the function of which is to restrain the exposure in the high density region of the original. Any substance, evincing actinic bleach-out behavior and having spectral absorption in the same general region as the diazo sulfonate, is suitable, for example, the diazo sulfonate used in the image-forming layer or any other light sensitive diazonium compound, such as those derived from p-phenylenediamines. If a diazo sulfonate be employed, the base may be coated on both sides with the hydrophobic resin and copolymer, the coatings rendered water sensitive, and the image bearing layer impregnated with the diazo sulfonate and a coupling component, and the layer on the other side with the diazo sulfonate. The same procedure may be followed if a different bleachable diazo be used, such as a diazo from a p-phenylenediamine, i. e., the diazo from N-diethyl-p-phenylenediamine, N-methyl-N-butyl-p-phenylenediamine and the like, in which case, such diazo is located in the layer opposite the image-forming layer. Conversely, the bleachable material may be located as a separate filter over the image-forming layer. In these modifications, exposure of the image-forming layers is effected through the bleachable layer.

The versatility of our diazo sulfonate foil is further

emphasized by the fact that it may be used to secure halftone dot transparencies from continuous tone transparencies by resorting to the use of contact screens such as those described in U. S. Patents 2,311,071; 2,478,433 and 2,478,444. Basically, these screens consist of an undulated density pattern on a very fine scale which, when interposed between an original and a reproducing medium of moderately high contrast, serve to break up the continuous tone pattern of the original into a corresponding "halftone" dot pattern in the reproduction. Excellent results are secured when a contact screen is interposed between a continuous tone original and a sheet of our negative foil, followed by exposure in an "Ozalid" machine or a vacuum frame. Positive halftone copies of a continuous tone negative original result. If desired, it is possible to combine such contact screens with the gradation controlling bleach-out layer previously discussed.

The invention will be further illustrated by the following examples, but it is to be understood that these are exemplary and not limitative.

#### Example I

A cellulose acetate base is coated by a Bird film applicator with the following solution:

6 grams polyvinyl methyl ether-maleic anhydride copolymer  
14 grams cellulose acetate (Hercules grade L-L1)  
30 grams methyl Cellosolve  
210 cc. acetone

After drying, the layer is passed over ammonia vapors several times, aired, and then sensitized from a water solution of the following:

4.8 grams sodium p-methoxybenzene diazo sulfonate  
3 grams o-sulfonylbenzaldehyde sodium salt  
3.5 grams phloroglucinol  
2 grams isopropanol  
Dilute to 100 cc. with water

After exposure to ultraviolet through a negative original for 1 to 3 minutes, depending upon the strength of the light source, followed by ammonia development, a sepia image is formed. After a 1 to 2 minute wash in warm water, numerous reprints of good quality may be made with little or no degeneration of the intermediate.

#### Example II

A cellulose triacetyl base is coated with the following solution by means of a reverse roll applicator:

2.5 grams polyvinyl isobutyl ether-maleic anhydride copolymer  
2.5 grams polyvinyl acetate (medium viscosity)  
35 cc. butyl acetate  
5 cc. methyl Cellosolve

Hydrolysis of the layer was effected by immersion in a 3% dilute solution of ethanolamine with subsequent doctoring of the excess solution. The sensitizing solution is as follows:

6 grams sodium p-ethoxybenzene diazo sulfonate  
4 grams resorcinol  
0.25 gram phloroglucinol  
1 gram citric acid  
1 gram sulfosalicylic acid  
4 grams zinc chloride  
4 grams thiourea  
0.1 gram isopropanol  
100 cc. water

After exposure and processing as in Example I, a deep sepia image is obtained. Copies of excellent maximum density may be made from this foil.

#### Example III

The same procedure is followed as in Example II, while using the following coating solution:

5 20 grams polyvinyl methyl ether-maleic anhydride copolymer  
20 grams cellulose acetate  
342 cc. acetone  
36 cc. methyl Cellosolve

10 The sensitizing solution was that of Example II with a 3% solution of 1-(5-hydroxy-1-naphthyl)biguanide substituted for the resorcinol and phloroglucinol. A reddish-brown image of excellent opacity results.

#### Example IV

A cellulose acetate base of combined acetic acid content of 60 to 60.9% is coated with the following organic solvent solution:

20 70 cc. acetone  
10 cc. methyl Cellosolve  
20 cc. denatured ethanol  
3 grams cellulose acetate combined acetic acid 55-56%  
3 grams polyvinyl methyl ether-maleic anhydride copolymer

25 The coated side of the base is then brought into contact with a 10% aqueous solution of 28° Baumé ammonia which reacts with the maleic anhydride effecting an opening and partial amidification of the anhydride  
30 rendering the coating hydrophilic. The excess of ammonia is wiped off and the base is then passed through a drying channel to drive off the residual water and ammonia.

The hydrophilic coating is then overcoated with a sensitizing solution compounded as follows:

35 8 grams sodium salt of p-ethoxybenzene diazo sulfonic acid  
4 grams zinc chloride  
0.5 gram sulfosalicylic acid  
4 grams thiourea  
4 grams tetrahydroxybiphenyl  
0.5 cc. of the product sold as "Aerosol MA" 70% by the American Cyanamid Company  
Water to a total of 100 cc.

45 The excess solution was wiped off with an air knife and the base is passed through a drying channel to remove residual water.

The foil is processed by placing a transparent or translucent line or continuous tone original over the sensitized foil and exposing by means of a suitable ultraviolet source. Those portions which are light struck are converted into the diazo which, when passed through a developing chamber containing ammonia, couples with the tetrahydroxybiphenyl to produce red-orange dye images. The foil is then washed with water to leach out the undecomposed diazo sulfonate thus fixing the image.

A positive image is obtained from a negative original and vice versa.

60 In the preceding examples, the molecular weight of the vinyl ether-maleic anhydride copolymer is normally such that a solution of 1 gram of the copolymer in 100 grams of 2-butanone has a viscosity of about 3 at 25°

65 C. Higher and lower molecular weights, however, can be used successfully with due attention to solvent balance, components of the solution and the coating method used.

The preparation of the water sensitive layers of the 70 type contemplated for use herein as a carrier for the sensitizing components is described in U. S. Patent 2,756,163 granted July 24, 1956. It is to be understood that any of the techniques referred to in such application may be employed in our invention.

75 It is to be equally emphasized that our invention is

grounded on the discovery that the use of the water sensitive layers of the prior application as a carrier for diazo sulfonates permits for the first time the commercial development of a stable satisfactory negative working diazo sulfonate foil.

*Example V*

A cellulose acetate base of combined acetic acid content of 60 to 60.9% is coated on both surfaces with the following organic solvent solution:

|                                                             |                             |
|-------------------------------------------------------------|-----------------------------|
| 20 grams polyvinyl methyl ether-maleic anhydride co-polymer | 10                          |
| 20 grams cellulose acetate                                  | 8 grams zinc chloride       |
| 342 cc. acetone                                             | 0.25 gram phloroglucinol    |
| 36 cc. methyl Cellosolve                                    | 2 grams sulfosalicylic acid |

Each coated surface of the base is then brought into contact with a 10% aqueous solution of 28° Baumé ammonia to render each coated side hydrophilic. The excess of ammonia is wiped off and the base is dried to remove residual water and ammonia.

One surface of the base, which may be referred to as the image side, is then overcoated with the sensitizing solution of Example IV. The opposite surface, which may be termed the back side, is coated with an 8% solution of the sodium salt of p-ethoxybenzene diazo sulfonic acid.

The foil thus produced is processed by placing a transparent or translucent line original over the back side of the sensitized foil and exposing by means of a suitable ultraviolet source. The portions of the foil which are light struck are converted into the diazo which, when passed through a developing channel containing ammonia, couples with the tetrahydroxybiphenyl to produce a red-orange image. The foil is then washed with water to leach out the undecomposed diazo sulfonate to fix the image.

By exposing the double coated foil in the indicated manner the exposure in the high density region of the original is suppressed. In this way, the low density contrast of the foil is materially increased.

*Example VI*

The negative working foil produced in accordance with Example IV is exposed to a continuous tone pattern between which and the foil is interpolated a contact screen prepared according to U. S. P. 2,311,071. By working up the foil as in Example IV, there is obtained a halftone dot pattern of the original.

*Example VII.—Preparation of continuous tone prints*

A piece of high acetyl cellulose acetate filmbase is pretreated by dip coating with a lacquer of the following composition and dried:

|                                                              |                                                                                       |
|--------------------------------------------------------------|---------------------------------------------------------------------------------------|
| 4.5 grams polyvinyl methyl ether-maleic anhydride co-polymer | 55                                                                                    |
| 4.5 grams cellulose acetate (56.5% acetyl, Hercules L-L1)    | 5.2 grams resorcinol                                                                  |
| 100 cc. acetone                                              | 1.6 grams 6,7-dihydroxynaphthalene-3-sulfonic acid, sodium salt                       |
| 40 cc. ethyl alcohol                                         | 0.4 grams 2,3-naphthalenediol                                                         |
| 20 cc. methyl Cellosolve                                     | 4 grams N,N-diethyl-4-amino-3-ethoxybenzene diazonium chloride, zinc chloride complex |
| 200 cc. acetone                                              |                                                                                       |

In order to reduce curl, the back side of the pretreated filmbase is dip coated with a solution of the following composition and dried:

|                                 |                                                                                                                                                                                                                                                                                                                                                                                                                                                                               |
|---------------------------------|-------------------------------------------------------------------------------------------------------------------------------------------------------------------------------------------------------------------------------------------------------------------------------------------------------------------------------------------------------------------------------------------------------------------------------------------------------------------------------|
| 55 cc. acetone                  | 65                                                                                                                                                                                                                                                                                                                                                                                                                                                                            |
| 40 cc. methanol                 | It should be noted that the materials cited must be used in the order given. For instance, if instead of the order—silver negative→diazo sulfonate intermediate positive→positive working diazo material—the order of the steps is changed to silver negative→positive working diazo material→diazo sulfonate foil, it will be found in the latter case that the contrast is excessive in the region of the middle tones and the overall continuous tone properties are poor. |
| 5 cc. methyl Cellosolve acetate | 70                                                                                                                                                                                                                                                                                                                                                                                                                                                                            |

The surface is rendered water sensitive by applying the following hydrolyzing solution by an applicator roll

75 with a 15 second imbibition time and with the excess thereafter doctoring off by means of a rubber bar:

|                    |   |
|--------------------|---|
| 5 cc. ethanolamine | 8 |
| 0.1 gram saponin   |   |
| 100 cc. water      |   |

The water sensitive surface next is sensitized with a sensitizing solution of the following composition:

|                                                 |                                                 |
|-------------------------------------------------|-------------------------------------------------|
| 60 cc. water                                    | 10                                              |
| 8 grams zinc chloride                           | 8 grams zinc chloride                           |
| 0.25 gram phloroglucinol                        | 0.25 gram phloroglucinol                        |
| 2 grams sulfosalicylic acid                     | 2 grams sulfosalicylic acid                     |
| 4 grams thiourea                                | 4 grams thiourea                                |
| 4 grams resorcinol                              | 4 grams resorcinol                              |
| 0.1 gram saponin                                | 0.1 gram saponin                                |
| 8 grams sodium p-methoxybenzene diazo sulfonate | 8 grams sodium p-methoxybenzene diazo sulfonate |
| 100 cc. water                                   | 100 cc. water                                   |

A positive print is prepared by exposing the foregoing sensitized surface beneath a normal negative in a machine, sold by General Aniline & Film Corporation under the trademark "Ozalid," at roughly 4 feet per minute, developed thoroughly with ammonia and fixed by washing in water for 1 to 3 minutes at a temperature of about 100° F. The surface can immediately be wiped dry by a cloth or cellulose towel and can be used immediately for producing further prints.

Thus, good black line continuous tone prints can be produced by reprinting the foregoing exposed and fixed foil onto a high brightness paper lacquered with a thin cellulose acetate dope, dried, and then sensitized with a solution of the following composition:

|                                                                                       |                                                                                       |
|---------------------------------------------------------------------------------------|---------------------------------------------------------------------------------------|
| 55 cc. water                                                                          | 30                                                                                    |
| 25 cc. isopropanol                                                                    | 5 cc. γ-valerolactone                                                                 |
| 5 cc. n-butyl alcohol                                                                 | 5 cc. n-butyl alcohol                                                                 |
| 5 cc. 85% formic acid                                                                 | 5 cc. 85% formic acid                                                                 |
| 2 grams anhydrous citric acid                                                         | 2 grams anhydrous citric acid                                                         |
| 2 grams thiourea                                                                      | 2 grams thiourea                                                                      |
| 1 gram zinc chloride                                                                  | 1 gram zinc chloride                                                                  |
| 5.2 grams resorcinol                                                                  | 5.2 grams resorcinol                                                                  |
| 1.6 grams 6,7-dihydroxynaphthalene-3-sulfonic acid, sodium salt                       | 1.6 grams 6,7-dihydroxynaphthalene-3-sulfonic acid, sodium salt                       |
| 0.4 grams 2,3-naphthalenediol                                                         | 0.4 grams 2,3-naphthalenediol                                                         |
| 4 grams N,N-diethyl-4-amino-3-ethoxybenzene diazonium chloride, zinc chloride complex | 4 grams N,N-diethyl-4-amino-3-ethoxybenzene diazonium chloride, zinc chloride complex |

The resulting print material is exposed beneath the diazo intermediate continuous tone foil at a speed of about 6 feet per minute on an "Ozalid" machine and developed with ammonia. The resulting prints exhibit improved continuous tone behavior in both the highlight and shadow regions.

Instead of sensitizing a cellulose acetate coated print material with the last formulation given, it is possible to sensitize a transparent foil with substantially this same formulation. Diapositives made on this material, using the intermediate diazo sulfonate foil, likewise exhibit smooth continuous tone behavior in the highlight and shadow regions.

It should be noted that the materials cited must be used in the order given. For instance, if instead of the order—silver negative→diazo sulfonate intermediate positive→positive working diazo material—the order of the steps is changed to silver negative→positive working diazo material→diazo sulfonate foil, it will be found in the latter case that the contrast is excessive in the region of the middle tones and the overall continuous tone properties are poor.

*Example VIII.—Preparation of prints with high contrast*

The procedure is similar to that of Example IV, excepting that the original negative is printed onto a high contrast positive working diazotype foil which, in turn, is printed onto the negative working diazo sulfonate foil

and the latter onto a positive working light sensitive material.

The positive working diazotype material on which the original negative is printed may, for example, be a product, such as is sold by General Aniline & Film Corporation under the trademark "Ozalid" Litho Foil 501 LC. This material comprises a cellulose acetate base sensitized with a diazo from a p-phenylenediamine and a phenolic coupler. It is to be emphasized, however, that any other high contrast positive working diazotype foil may be used.

By proceeding as in Example IV, the diazo sulfonate foil may be printed onto either a positive light sensitive diazotype material, such as that indicated above, or upon a positive photographic film with the sensitive surfaces of the foil and positive material in contact. The prints resulting from this procedure are notable for their exceedingly high contrast.

It is believed to be evident that in lieu of the light sensitive positive working diazotype material on which the negative working foil is printed as described above, any other positive working light sensitive diazotype film or paper may be used with equally good results. Examples of such materials, for instance, are given in U. S. application, Serial No. 350,528 filed by Peter T. Woitach, Jr., on April 22, 1953, now abandoned, and U. S. Patent No. 2,709,655 granted May 31, 1955.

Various modifications of the invention will be apparent to those skilled in the art and we, therefore, do not intend to be limited in the patent granted except as necessitated by the appended claims.

We claim:

1. A negative working diazo sulfonate material comprising a transparent base carrying a layer of a mixture of a copolymer of maleic anhydride with a vinyl compound and a hydrophobic resin compatible with said copolymer, said copolymer having been surface hydrolyzed with a moist water soluble nitrogenous base to render it hydrophilic and a light sensitive diazo sulfonate in which the sulfonate group is directly attached to a nitrogen atom of the azo group and a coupling component imbibed to said layer.

2. The product as defined in claim 1, wherein the vinyl compound is a vinyl ether.

3. The product as defined in claim 1, wherein the vinyl compound is a vinyl aliphatic ether.

4. The product as defined in claim 1, wherein the ratio

of copolymer to hydrophobic resin by weight is from 1:6 to 6:1.

5. The product as defined in claim 1, wherein the hydrophobic resin is a cellulose ester.

6. The product as defined in claim 1, wherein the vinyl compound is a vinyl ether and the molecular weight of the copolymer is such that a solution of 1 gram thereof in 100 grams of 2-butanone has a viscosity of about 3 at 25° C.

10 7. The product as defined in claim 1, wherein the diazo sulfonate is p-ethoxybenzene diazo sulfonate, and the coupling component is a polyhydric phenol.

8. A negative working diazo sulfonate material comprising a transparent base carrying a layer of a mixture of a copolymer of maleic anhydride with a vinyl compound and a hydrophobic resin compatible with said copolymer, said copolymer having been surface hydrolyzed with a moist water soluble nitrogenous base to render it hydrophilic, a light sensitive diazo sulfonate in which the sulfonate group is directly attached to a nitrogen atom of the azo group and a coupling component imbibed to said layer and a filter layer containing a compound bleachable by actinic light through which the sensitized surface is exposed.

20 9. A negative working diazo sulfonate material comprising a transparent base, each surface of which carries a layer of a mixture of a copolymer of maleic anhydride with a vinyl compound, and a hydrophobic resin compatible with said copolymer, said copolymer having been surface hydrolyzed with a moist water soluble nitrogenous base to render it hydrophilic, a light sensitive diazo sulfonate in which the sulfonate group is directly attached to a nitrogen atom of the azo group and a coupling component imbibed to the layer of one surface and a diazo compound bleachable by actinic light imbibed to said other surface.

#### References Cited in the file of this patent

#### UNITED STATES PATENTS

|           |                        |               |
|-----------|------------------------|---------------|
| 2,156,069 | Schlack -----          | Apr. 25, 1939 |
| 2,197,456 | Von Poser et al. ----- | Apr. 16, 1940 |
| 2,699,392 | Herrick et al. -----   | Jan. 11, 1955 |

#### FOREIGN PATENTS

|         |                     |              |
|---------|---------------------|--------------|
| 402,737 | Great Britain ----- | Mar. 5, 1942 |
|---------|---------------------|--------------|